

## UNITED STATES PATENT OFFICE

GEROULD T. LANE, OF ROCHESTER, NEW YORK, ASSIGNOR TO EASTMAN KODAK COMPANY, OF ROCHESTER, NEW YORK, A CORPORATION OF NEW YORK

## SIZED PAPER AND METHOD OF MAKING SAME

No Drawing. Continuation of application Serial No. 318,995, filed November 12, 1928. This application filed March 1, 1929. Serial No. 343,838.

This invention relates to a new and improved method for the manufacture of engine or beater sized paper.

It has hitherto been impossible to manufacture from any fiber, however purified, an engine or beater sized paper having great durability, that is, a paper that does not deteriorate or oxidize with age. One test or effect of the oxidation or degeneration of the paper is that if a sensitive photographic emulsion is left in contact with the paper, particularly under humid or heated conditions, the emulsion will on development show fog, evidently the result of such oxidation. This may be utilized as a measure of the oxidation. The formation and presence of considerable such fog obviously renders a paper unfit for use for photographic purposes, either as a support for sensitive layers or as a wrapping material for sensitive goods.

I have discovered that purified paper pulp if treated in the beater with a soap made from a saturated fatty acid so pure as to have a low iodine number, and particularly from the fatty acids of high molecular weight, in the presence of an acid or acid salt will have precipitated thereon a size in the presence of which the fiber does not become oxidized or degenerated.

The fiber can be any cellulose of high alpha-cellulose content, preferably greater than ninety per cent. Wood pulp fiber purified to the above extent gave the best results, as a greater degree of sizing was obtained with its use.

Any saturated fatty acids capable of being saponified, whether obtained from waxes, fats, or produced synthetically by hydrogenation of unsaturated compounds, can be used in this process if they have been freed from unsaturated compounds so that they have a low iodine number. Fatty acids of higher molecular weight give the best results for sizing purposes.

For various practical reasons such as cost the most available are palmitic and stearic acids. The ordinary commercial acids usually include other unsaturated acids and have, therefore, a higher iodine value than five by the Hanus method as described in pages

286-287 and 288 sections 17 and 18 of The Official and Tentative Methods of Analysis of the Association of Official Agricultural Chemists, second edition, and should be purified by the eliminating of those unsaturated acids, such as oleic acid, or other easily oxidized material. Stearic acid known commercially as triple pressed stearic acid is satisfactory.

The known natural waxes include saturated and unsaturated compounds and when utilized for the sizing of papers do not protect the fibers from deterioration. However, by the removal of the unsaturated and oxidizable compounds the saturated acids of the waxes may be rendered available.

The iodine number is a measure of the extent to which the material will take up oxygen and is, therefore, a very useful determinant of the extent to which the fiber will later deteriorate or oxidize in the presence of the size.

It may be noted that ordinary resin size such as is customarily used has an iodine number of 80 or more and the paper pulp treated with it rapidly deteriorates. A high grade white toilet soap made from mixed acids of a quality easily obtainable on the market has an iodine value of the order of 40 and gives better results but not sufficiently good for most photographic purposes or for indefinite durability. A chemically pure fatty acid would have an iodine number of zero but would be too expensive for large scale production. A paper made with soap having an iodine number of less than 20 will be stable enough for most purposes. If the number is greater than 80, the deterioration is undesirably great. Oleic acid, a very common impurity in the higher fatty acids, has an iodine number of ninety and hence its presence in the quantity frequently found in commercial soaps and acids is very undesirable.

As a working example of my process, the following is typical: Paper pulp, or more especially purified sulphite pulp, of extremely high alpha cellulose content, that is over 90%, is furnished in the ordinary way to the beater. One to three per cent, based on the

weight of the pulp, of triple pressed commercial stearic acid is saponified with a chemically equivalent amount of caustic soda, or other alkali. This is added to the pulp in 5 the beater and is precipitated on the fiber by sufficient of a solution of aluminum sulphate to completely neutralize the alkalinity of the soap. The amount added would, of course, depend upon the particular acid or 10 alkaline condition of the beater contents, such as the hardness of the water used, the amount and alkalinity of the soap and the acid or alkaline state of the cellulose fiber itself. It is comparatively immaterial in 15 what order the soap and the acid are added or at what point in the beating operation. The other operations of the paper making follow standard practice.

Any acid or acid salt capable of precipitating 20 the size upon the paper fiber may be used instead of aluminum sulfate; particularly potassium, ammonium or chrome alum or other sulfates such as magnesium or copper sulfate.

25 Commercial stearic acid, even when pressed, still contains a considerable proportion of palmitic acid which is satisfactory for my purposes.

The product made as above described can 30 be differentiated from other sized papers by its non-fogging action on photographic plates or emulsions when placed in contact therewith for a long period of time under ordinary conditions or for shorter periods 35 of time when incubated at 120° F. or above. In general, this fogging action is increased by exposure of the paper to be tested, which is, of course, unsensitized, to light prior to the test. On the subsequent development of 40 the photographic plate or emulsion there is produced a fog which is a measure of, and is presumably proportional to, the oxidation or deterioration that took place in the paper during the test. This plate test is in fact a 45 convenient and satisfactory method of measuring the useful life or lasting quality of any paper.

Heretofore no paper has been made for photographic or other uses, requiring a beater sized paper, that would not affect the 50 quality of the sensitized coating on account of the oxidation or deterioration taking place in the paper, or that would not yellow and deteriorate itself.

55 Paper made by my improved process and subjected to a severe test of the type outlined, results in no detectible fog on the developed photographic plate and is, therefore, admirably adapted for photographic or other purposes where permanency and non-fogging qualities are pre-eminently desirable.

This process is of the utmost value from a 60 practical standpoint for with its use a paper can be produced of the greatest durability and with no deteriorating effect when near

or in contact with sensitized photographic emulsions. Also owing to the fact that the best sizing results are obtained when this process is used with sulphite pulp, a paper can be made by this process using purified 70 sulphite pulp of an alpha-cellulose content greater than 90% which is more durable than any beater-sized paper produced from linen or cotton or any other fiber of which I have knowledge. 75

The paper produced has improved strength and flexibility, has a fine smooth surface, and high resistance to chemicals, moisture, oily substances, heat, light and combinations of these elements. Not only 80 is it remarkably better in these qualities than sulphite or rag papers made with rosin sizing, but it is even more permanent than papers containing no beater sizing, owing to the protection afforded the fibers 85 from air and moisture by the precipitated fatty acid. This improved sizing, being water repellent, gives greater protection than materials which are not water repellent or are more or less water permeable or soluble, 90 such as glue, gelatine, starches or other similar materials.

I contemplate as included in my invention all such modifications and equivalents as fall 95 within the scope of the appended claims. 95

This application is a continuation of my application Serial No. 318,995, filed November 12, 1928.

Having thus described my invention, what I claim as new and desire to secure by Letters 100 Patent is:

1. In the process of making paper, the step that includes precipitating on the fibers while in a pulp condition a sizing from a soap of a saturated fatty acid containing more than nine carbon atoms and purified to an extent such that its iodine number is less than 40. 105

2. In the process of making paper, the step that includes precipitating on the fibers while in a pulp condition a sizing from a soap of a saturated fatty acid containing more than nine carbon atoms and purified to an extent such that its iodine number is less than 20. 110

3. In the process of making paper, the step that includes precipitating on the fibers while in a pulp condition a sizing from a soap of a saturated fatty acid containing more than nine carbon atoms and purified to an extent such that its iodine number is less than 5. 115

4. In the process of making paper, the step that includes precipitating on the fibers of sulphite paper pulp having an alpha-cellulose content greater than ninety per cent, a sizing from a soap of a saturated fatty acid containing more than nine carbon atoms and purified to an extent such that its iodine number is less than 40. 120

5. In the process of making paper, the step that includes precipitating on the fibers of sulphite paper pulp having an alpha-cellulose 125

content greater than ninety per cent, a sizing from a soap of a saturated fatty acid containing more than nine carbon atoms and purified to an extent such that its iodine number is less than 20.

5 6. In the process of making paper, the step that includes precipitating on the fibers of sulphite paper pulp having an alpha-cellulose content greater than ninety per cent, a sizing from a soap of a saturated fatty acid containing more than nine carbon atoms and purified to an extent such that its iodine number is less than 5.

10 7. In the process of making paper that includes sizing in the beater, the step of adding to the paper pulp during such beating the soap of a saturated fatty acid containing more than nine carbon atoms and having an iodine number less than 40, and a precipitant for such soap.

15 8. In the process of making paper that includes sizing in the beater, the step of adding to the paper pulp during such beating the soap of a saturated fatty acid containing more than nine carbon atoms and having an iodine number less than 20, and a precipitant for such soap.

20 9. In the process of making paper that includes sizing in the beater, the step of adding to the paper pulp during such beating the soap of a saturated fatty acid containing more than nine carbon atoms and having an iodine number less than 5, and a precipitant for such soap.

25 35 10. In the process of making paper that includes sizing in the beater, the step of adding to the paper pulp during such beating the soap of a higher saturated fatty acid containing more than nine carbon atoms and so free from unsaturated compounds that its iodine number is less than 40, and a precipitant for such soap.

40 45 11. In the process of making paper that includes sizing in the beater, the step of adding to the paper pulp during such beating the soap of a higher saturated fatty acid containing more than nine carbon atoms and so free from unsaturated compounds that its iodine number is less than 20, and a precipitant for such soap.

50 55 12. In the process of making paper that includes sizing in the beater, the step of adding to the paper pulp during such beating the soap of a higher saturated fatty acid containing more than nine carbon atoms and so free from unsaturated compounds that its iodine number is less than 5, and a precipitant for such soap.

60 13. As an article of manufacture, paper comprising cellulose fibers individually coated with a material precipitated from the soap of a saturated fatty acid containing more than nine carbon atoms and so purified that its iodine number is less than 40.

65 14. As an article of manufacture, paper

comprising cellulose fibers individually coated with a material precipitated from the soap of a saturated fatty acid containing more than nine carbon atoms and so purified that its iodine number is less than 20.

70

15. As an article of manufacture, paper comprising cellulose fibers individually coated with a material precipitated from the soap of a saturated fatty acid containing more than nine carbon atoms and so purified that its iodine number is less than 5.

75

16. As an article of manufacture, paper comprising sulfite pulp fibers individually coated with a material precipitated from the soap of a saturated fatty acid containing more than nine carbon atoms and so purified that its iodine number is less than 40.

80

17. As an article of manufacture, paper comprising sulfite pulp fibers individually coated with a material precipitated from the soap of a saturated fatty acid containing more than nine carbon atoms and so purified that its iodine number is less than 20.

85

18. As an article of manufacture, paper comprising sulfide pulp fibers individually coated with a material precipitated from the soap of a saturated fatty acid containing more than nine carbon atoms and so purified that its iodine number is less than 5.

90

19. As an article of manufacture, paper comprising sulfite pulp fibers having an alpha cellulose content greater than ninety per cent and individually coated with a material precipitated from the soap of a saturated fatty acid containing more than nine carbon atoms and so purified that its iodine number is less than 40.

95

20. As an article of manufacture, paper comprising sulfite pulp fibers having an alpha cellulose content greater than ninety per cent and individually coated with a material precipitated from the soap of a saturated fatty acid containing more than nine carbon atoms and so purified that its iodine number is less than 20.

100

21. As an article of manufacture, paper comprising sulfite pulp fibers having an alpha cellulose content greater than ninety per cent and individually coated with a material precipitated from the soap of a saturated fatty acid containing more than nine carbon atoms and so purified that its iodine number is less than 5.

110

22. As an article of manufacture, paper comprising sulfite pulp fibers having an alpha cellulose content greater than ninety percent and individually coated with a material precipitated from the soap of a saturated fatty acid of higher molecular weight and sufficiently free from unsaturated compounds that its iodine number is less than 40.

115

23. As an article of manufacture, paper comprising sulfite pulp fibers having an alpha cellulose content greater than ninety per cent and individually coated with a ma-

120

125

130

terial precipitated from the soap of a saturated fatty acid of higher molecular weight and sufficiently free from unsaturated compounds that its iodine number is less than 20.

**5** Signed at Rochester, New York this 22nd day of Feb., 1929.

**GEROULD T. LANE.**

**10****15****20****25****30****35****40****45****50****55****60****65**